

## 1

3,369,930

METAL PROCESSING COMPOSITIONS AND  
METHOD

Wesley J. Wojtowicz, Detroit, Mich., assignor to The H. A. Montgomery Company, Detroit, Mich., a corporation of Michigan  
No Drawing. Filed Dec. 6, 1963, Ser. No. 328,507  
18 Claims. (Cl. 117—134)

## ABSTRACT OF THE DISCLOSURE

As a metal working lubricant, a mixture of lubricating oil of 1,500—10,000 S.U.S. at 100° F. and a water-soluble organic amine soap of low titer fatty acid, blended in proportions of 34—75 parts of oil to 66—25 parts of soap by weight. A film of the lubricant composition of the invention, at a temperature of 50—400° F., is applied to metal stock with or without removal of previously applied "mill oil." Application may be effected by roll-coating, spraying, dipping, doctoring, or other means, roll-coating being preferred. After dissipation of any residual heat in the coating by exposure to ambient temperatures, the coated metal sheet is subjected to metal-working operations, such as deep-drawing, to form a fabricated article. Welding and painting of the deformed workpiece are performed without removing residual lubricant film; or the lubricant film may be removed by using conventional alkali or acid phosphate cleaners or vapor degreasers to expose polished surfaces of the metal.

Some of the prior compositions for coating metals prior to metal working operations required removal before major subassemblies of parts could be made therefrom because the prior coatings interfered with welding. It will be readily understood that a new process otherwise as good as such old process, but not requiring removal of the coating prior to welding, would provide a substantial advance in the art.

Should the later development also make it possible to store components for extended periods without corrosion—prior to making the welded sub-assembly—the advantages over the prior art would be still greater.

A still further advance in the art would be provided by a deep-draw lubricant that embodied all of the favorable characteristics of the prior art but, additionally, was compatible with primer paints and, therefore, need not be removed at all in the course of converting the welded subassembly into a finished, painted product.

A general object of the present invention is to provide a novel deep-draw formulation for the metal processing industry and a new procedure for using such formulation.

More specific objects are to provide a novel, deep-draw, metalworking composition that provides a coating for metals, the coating having the following characteristics:

- (a) adhesiveness to metal surfaces, obviating pre-cleaning;
- (b) lubrication of both the metal surface and the draw dies for metalworking operations;
- (c) compatibility with additional die lubricants for deep-drawing and the like;
- (d) requiring no heat for drying the applied coating;
- (e) provision of corrosion protection during extended storage of deep-drawn parts;
- (f) no interference with welding of drawn parts; and
- (g) no interference with painting of drawn parts.

A further object is to provide an improved article of manufacture, to wit, a metal surface having a coating

## 2

thereon which protects it before, during and, after cold-working.

## THE COMPOSITIONS OF INVENTION

5 Compositions made in accordance with the present invention, for producing the coatings of the invention, are non-aqueous. They consist essentially of a lubricating oil having a viscosity in the range of 1,500 to 10,000 S.U.S. at 100° F. and a water-soluble alkanol amine 10 soap of low titer fatty acid in proportions of 34—75 parts of oil to 66—25 parts of amine soap, by weight. A typical composition would comprise the following:

| Ingredient:                         | Percent by weight |
|-------------------------------------|-------------------|
| Mineral oil, 5000 S.U.S. at 100° F. | 66                |
| Organic amine soap                  | 34                |

The character of both the oil and the soap is further defined below.

20 Preparation of the above composition merely requires blending the ingredients in the amounts indicated at ambient temperatures. The physical appearance of the product so produced is a heavy, highly viscous, grease-like material.

25 Application of such composition to a metal surface may be by roll-coating, spraying, dipping, doctoring, or other procedure at a suitable temperature for the particular application procedure in the range from 50—400° F., elevated temperatures being employed to reduce the viscosity as needed for the particular application procedure employed. Residual heat in the applied coating is permitted to dissipate by radiation at ambient temperature.

30 *Mineral oil.*—An effect of this material is to insolubilize the film and thus render it compatible with zinc-rich primer paints. This makes it possible to pain fabricated components, without the necessity of cleaning the film of the invention from such components prior to painting. It should be pointed out at this time that, by the present invention, the intrinsic salt spray resistance of the zinc-rich primer paints is not in the least affected by the coatings of the present invention. In fact, the present coatings preserve the nascent or raw state of the metal surface as it comes from the strip mill to the processor

35 for fabrication by deep-draw operation or the like. Thus, the adherence of the subsequently applied primer paint is substantially increased over application of such material to a partially oxidized surface that may have been exposed to the atmosphere prior to application of the primer paint.

40 The hydrocarbon or mineral oil set forth in the prior examples is a preferred component to be used in accordance with the present invention, primarily because of its low cost, ease of quality control, and ready availability in quantity. This material may have a viscosity in

45 the range of from about 1500 to 10,000 Saybolt Universal Seconds at 100° F. The lubricating qualities of the films of the invention increase with increasing viscosity of the oil phase. Localized hot spots which may occur on draw dies in deep-drawing operations are known to cause

50 failure of a lubricant film. The more viscous materials are desirable, therefore, because they are less sensitive to this temperature effect. The indicated upper viscosity limit of 10,000 S.U.S. at 100° F. is based only on problems encountered in application of the materials of invention. In the present invention, therefore, the lower limit is more carefully guarded to assure a safety factor, as required of materials capable of operating at elevated temperatures under high deep-drawing pressures.

55 Within the scope of the invention, a compounded vehicle, such as lighter weight oil containing an additive resin to increase the viscosity, can be employed. Specific

component materials within this category that have been successfully used are as follows:

Piccopale 70 (a non-registered mark designating a product of the Pennsylvania Industrial Chemical Corporation). This is a hydrocarbon resin with a color of G-10 on the Gardner scale. The material is available in solid, flaked, and solution form. It is soluble in all aliphatic hydrocarbons, aromatic hydrocarbons, chlorinated hydrocarbons, naval stores, most esters, ethers, and ketones, and some alcohols.

Stikvel W (a product of the Velsicol Chemical Corporation) is also applicable.

In some instances, a hydrogenated or bodied vegetable oil can be used as the vehicle of the present invention. Also esterified acids as used in the paint and varnish industry can be used.

The organic amine soaps: These materials can be prepared from any of the water-soluble alkanol amines and a fatty acid with a titer not exceeding 30° C. The "titer" of a soap may be defined as the solidifying point of the fatty acids liberated from a fat. The determination of this point by melting the acids in a tube and noting the temperature at which they solidify again on cooling is called the "titer test."

The amine soaps used in accordance with the present invention can be prepared using conventional soap-forming fatty acids having titers below about 30° C. These fatty acids may be mixtures of fatty acids derived from various oils, such as vegetable oils. For example, the acid mixtures derived from castor, coconut, palm kernel, linseed, olive, peanut, rapeseed, corn, and soya bean oils are suitable. Also suitable are the individual acids, such as oleic acid, ricinoleic acid, etc., which have been separated from fatty acid mixtures such as those mentioned above. In addition, fatty acids such as tall oil, which are formed as by-products from the manufacture of chemical wood pulp, can be used.

The amines, which are reacted with the low-titer fatty acids to form the amine soaps, may be any of the water-soluble, organic amines having boiling points above about 100° C., for example: ethylene diamine, monoethanolamine, diethanolamine, triethanolamine, dimethyl ethanolamine, monoisopropanol amine, morpholine, and 2-amino-1-butanol. Particularly advantageous for use in high speed roller coating processes are coating compositions in which the amine soap is made with amines such as 2-amino-2-methyl-1-propanol; 2-amino-2-methyl-1,3-propanediol; and 2-amino-2-ethyl-1,3-propanediol.

The coatings of the invention may be modified by the incorporation of selected materials. Thus, where the coated sheets are to be stacked for a period of time prior to fabrication, it may be desirable to incorporate an anti-blocking agent in the composition to minimize the sticking of one sheet to another. Suitable anti-blocking agents are those which are compatible with the coating compositions but which migrate to the surface of the coating to form a tack-free superficial film upon drying of or congealing of the film. An example is methyl cellulose and/or polyvinyl alcohol, when used in amounts by weight of from about 5-15% on an anhydrous basis.

The coating compositions of the invention also may be modified, if desired, by the addition of small amounts of other materials known to improve the drawing qualities of lubricants. These may include water-insoluble materials such as chlorinated oils, flowers of sulfur, colloidal graphite etc.

The compositions can be additionally compounded with water as a carrier, for application. When so operating, of course, the water must be removed after application, as by oven drying which has been common with aqueous coating materials of the past. This may be considered by some practitioners as a less desirable manner of operation than has been previously described relative to application of the coatings of invention in "neat" or non-aqueous form.

In the appended claims, it is not intended that the

presence of modifying agents or materials, such as those suggested above, be excluded by defining the compositions as "consisting essentially of" specified components.

The selection of a particular coating composition in accordance with the present invention is primarily dependent upon the fabricating operation which is subsequently to be performed on the metal, the deciding factor being the magnitude of the coefficient of friction between the workpiece and the tool used in the shaping thereof. One method for evaluating this lubricant property is described in an article entitled "Sliding Friction Test for Metalworking Lubricants" by W. J. Wojtowicz, published in the May and June, 1955 issues of Lubrication Engineering. For moderate metal drawing operations, lower soap contents may be used in the compositions of the invention within the range indicated above.

Film thickness ranges as used in the present invention can be defined in two ways, to wit:

(1) The films are applied in a thickness range of 100 to 200 milligrams per square foot of metal surface.

(2) Stated in terms of thousandths of an inch thickness, these will generally be in the following ranges, depending upon the severity of the metalworking operations to be encountered. The optimum coating thickness depends upon the gauge of the workpiece and the severity of the working operation, with heavier coatings being used for more difficult operations. Generally, coatings having a thickness in the range of 0.00003 to 0.001 inch are preferred. A good general average coating thickness for most metalworking operations is .0001 inch.

The compositions of the invention are applicable to the following metal surfaces:

- (a) Plain cold-rolled steel, having a brushed, polished or other surface thereon to be protected;
- (b) Stainless steel in various degrees of surface finish;
- (c) Aluminum;
- (d) Magnesium;
- (e) Brass and the like.

As indicated above, the workpieces or strip stock can be polished to a high lustre before the coating is applied, because these surface finishes are protected during subsequent handling, storage, and metalworking operations.

#### ADVANTAGES OF COMPOSITIONS AND COATING

The lubricating and protective films of the invention are readily compatible with many other die lubricants.

A particular advantage of the films produced by the present invention is that they do not contain any alkali soaps. Such are known to seriously detract from the salt spray resistance of a composite lubricant-zinc primer film. Therefore, by the absence of such materials from compositions of the present invention, the salt spray resistance of zinc-primer films is not weakened in the least. Currently used oil films are unsatisfactory in this respect because they do contain more than 5% of sodium or potassium soap. On the other hand, the pure organic amine soap-mineral oil compositions of this invention provide excellent compatibility without detracting from the salt spray resistance of zinc primer films.

Cleaning the films of the present invention from a coated workpiece after its fabrication is not necessary, particularly where painted surfaces are to follow. However, if this is for some reason required, as where a previously polished surface has been protected and is to be exposed in final application, cleaning can be easily performed. This is accomplished by conventional cleaning equipment already widely employed in connection with metal drawing operations. Thus, a combination of brushes with a hot spray or bath of cleaning solution, such as aqueous alkali, emulsion cleaners, acid phosphate cleaners, and vapor degreasers, will be found operable.

A further advantage of the formulations of the invention is that they resemble in physical properties many of

the previously used materials for the same purposes. Thus, equipment in existence can be used without modification or without substantial alteration, except, of course, for shutting down the drying ovens that probably are existent therein, from the use of the prior aqueous base materials.

#### APPLICATION OF COMPOSITIONS

It is believed that the method of applying the compositions of the invention can best be visualized by following, step by step, an exemplary strip of cold rolled steel through a protective coating operation and subsequent deforming step of the invention. It will be presumed that a surface of the strip is polished to receive paint in the fabricated form.

##### (I) Precleaning

Because the compositions of invention have an oil-like base, it will follow that they have a substantial degree of compatibility with oily protective coatings (mill oil), commonly applied to strip steel at the finishing mill. Therefore, due to this oil compatibility, it is not necessary that the metal surface be rendered absolutely oil-free prior to application of the present compositions thereto. If the surface of the metal contains large amounts of oil, the surface should be at least squeegeed or wiped to remove any excess prior to application of the coating composition. The metal surface is then ready for application in accordance with the present invention.

##### (II) Application

When treating strip stock, roll coating is highly desirable because the roll coater can operate in a heated bath of the material and pick up an appropriate load for application and thus control the thickness of film applied. A further advantage of roll coating is that it provides a method of applying the compositions of the invention without removing the prior protective oil film, and yet the application is of such nature that a tightly adherent lubricant film results when the present compositions are applied. As the roll applies the coating to the metal surface, it breaks through the existing oil film and mixes the oil and the coating composition in intimate combination. The coating composition, in turn, takes up the residual oil and makes it an integral part of the ultimate coating so that it will not interfere with the adhesion of the coating to the strip, as by acting like a parting material.

The thickness of the film applied to the strip is governed by control of the application viscosity or temperature of the composition at the point of application.

Although the compositions of the invention are particularly adapted for use in roller coating operations, they also provide several advantages when employed in other methods of coating, such as spraying or dipping. In general, the viscosity of the compositions, or temperature, will be varied to place them in a compatible range with the coating method employed. As an example, when used in the roller coating process, viscosities in the range of 1500 to 5000 S.U.S. at the temperature of application will generally be applicable. This generally connotes a temperature of application of from 150 to about 300° F. In the case of dip-coating, viscosities will generally be retained in the slightly lower range of 1500 to 2000 S.U.S. To effect these viscosities, application temperatures are approximately 200 to 250° F.

For spraying operations, it is not desired that the coating be heated because of the difficulty of retaining it in such condition as it passes through the lines, orifices, nozzles, and the like. Therefore, the naturally lower viscosity materials of 1500 to about 1800 S.U.S. at 100° F. are preferred for spraying.

Other methods of application, such as by a doctor blade, are not excluded from the scope of invention. By so operating, the compositions can be applied at room temperature, 60-90° F.

In summary, coating thicknesses can be controlled by

the method of applying the composition and by varying the viscosity of the composition at the situs of application; the greater the viscosity, the thicker the applied coating will be.

Relative to application, it is important where a surface is not chemically clean, as where it might contain a residual corrosion-protecting oil film, to press physically the composition into intimate contacting relationship with the surface to provide a tight bond. Thus, it can be said that the coating composition is physically admixed with any residual oil film on the surface of the metal.

##### (III) Exposure to ambient temperature

The composition and the metal are then exposed to ambient temperature so that the heat of the coating, if any, can be dissipated.

##### (IV) Subsequent processing

After the coatings of invention are applied, that is, immediately after drying or setting, the coated workpiece can be cold-worked by any usual procedure such as deep-drawing, shearing, form-rolling, and the like.

While cold-working metal workpieces, which is to be understood as including blanking, piercing, cutting, and perforating, the coatings have special value in that they effectively protect the tools or dies used to fabricate the workpiece, as well as the coated surfaces of the metal workpiece.

#### ADVANTAGES OF THE INVENTION

From the foregoing, it can be understood that several advantages arise from the use of the present invention. One is that, particularly when using the roller coating application technique, the metal sheets do not have to be chemically clean for satisfactory operation. This is in direct contrast to the old dry lubricant coating processes where it was not only necessary to thoroughly clean the sheets prior to coating, but also to make sure that any cleaning agent on the sheets was removed prior to application of the dry coating.

Thus, all alkali washing materials, phosphates, tanks and the like are replaced perhaps by a simple swab or equivalent wiping device.

Another advantage flowing from the invention of particular importance is its application in highly automated production lines in which metal sheets or continuous strips are moved substantially continuously at a relatively high rate of speed from a supply point or reel and through a coating, drying, and single or plural-stage fabricating operation, all without marring the surface finish previously applied to the strip at the finishing mill.

A further advantage of the present invention resides in the fact that drying of the applied coating, as by heating in an oven or the like, is not required. It will be observed that substantial reduction in expense is encountered by so operating. Both the cost of the fuel to fire such an oven and the capital investment of the oven are obviated.

A further advantage is that substantially reduced plant areas of operation are required for effecting the present invention because of the omission of the following components from a floor space area:

- (a) Precleaning equipment, which is either eliminated or substantially reduced in physical size to a wiping squeegee and collection tank for excess mill oil wiped from the workpiece; and
- (b) The oven and the associated fueling system therefor.

Since the process of the invention is readily integrated into existing equipment, generally by the mere closing down or removal of the pre-cleaning and oven components thereof, metal fabricators can effect an immediate savings in their operations and produce better products because of the inherent advantages of the films of invention.

From the foregoing, it will be understood that the present invention provides coatings, compositions, and a process for effectively protecting finished metal work surfaces prior to and during cold working operations with a high degree of flexibility for adapting the invention to a variety of metalworking operations and metals to be worked, and for integrating the process of the invention into existing production lines with minimum modification of existing equipment.

What is claimed is:

1. A coating composition consisting essentially of the following ingredients blended in the range of proportions indicated:

Ingredient: Parts by weight  
Lubricating oil, 1,500-10,000 S.U.S. at  
100° F. 34-75  
Water-soluble organic amine soap of low titer  
fatty acid 66-25

2. A coating composition according to claim 1 in which the lubricating oil is a mineral oil.

3. A coating composition according to claim 1 in which the lubricating oil is a vegetable oil.

4. A coating composition according to claim 1 in which the soap-forming organic amine is a water-soluble aliphatic amine.

5. A coating composition according to claim 1 in which the soap-forming organic amine is a water-soluble alkanol amine.

6. A coating composition according to claim 1 in which the soap-forming organic amine has a boiling point above about 100° C.

7. A metal workpiece having on its surface a coating of a composition consisting essentially of the following ingredients blended in the range of proportions indicated:

Ingredient: Parts by weight  
Lubricating oil, 1,500-10,000 S.U.S. at  
100° F. 34-75  
Water-soluble organic amine soap of low titer  
fatty acid 66-25

said coating being present in the amount of about 100-200 milligrams per square foot of metal surface area.

8. A coated metal workpiece according to claim 7 in which the lubricating oil of the coating composition is a mineral oil.

9. A coated metal workpiece according to claim 7 in which the lubricating oil of the coating composition is a vegetable oil.

10. A coated metal workpiece according to claim 7 in which the soap-forming organic amine is a water-soluble aliphatic amine.

11. A coated metal workpiece according to claim 7 in which the soap-forming organic amine is a water-soluble alkanol amine.

12. A coated metal workpiece according to claim 7 in which the soap-forming organic amine has a boiling point above about 100° F.

13. The method of forming a lubricant coating over an oil-coated surface of a metal workpiece comprising the steps of wiping any excess oil from said surface as required to leave only a thin film thereof, applying over said thin oil film a coating composition consisting essen-

tially of the following ingredients blended in the range of proportions indicated:

Ingredient: Parts by weight  
5 Lubricating oil, 1,500-10,000 S.U.S. at  
100° F. 34-75  
Water-soluble organic amine soap of low titer  
fatty acid 66-25

and physically pressing said coating composition into intimate contacting relationship with said thin oil film to effect integration of the latter with the coating composition and bonding of the resulting integrated composition to the metal surface.

14. The method of forming a lubricant coating according to claim 13, in which method said coating composition is applied in a heated condition at a temperature in the range of 50-350° F. and, after its application, is cooled by exposure to ambient temperature.

15. In the processing of a metal workpiece to form a fabricated article, the steps of—

(a) Applying to a surface of a workpiece an adherent film of a metalworking lubricant consisting essentially of the following ingredients blended in the proportions indicated:

20 Ingredient: Parts by weight  
Lubricating oil, 1,500-10,000 S.U.S. at  
100° F. 34-75  
Water-soluble organic amine soap of low titer  
fatty acid 66-25

(b) Deforming the coated workpiece between metalworking dies while said adherent film serves as a lubricant between the workpiece and the dies; and

(c) Without removing residual amounts of said adherent film remaining on the deformed workpiece, completing the fabricated article by performing finishing operations thereon.

16. In the processing of a metal workpiece to form a fabricated article, the steps of claim 15, wherein a primer paint coating is applied to the deformed workpiece as a finishing operation without first removing residual amounts of said adherent film from the deformed workpiece.

17. In the processing of a metal workpiece to form a fabricated article, the steps of claim 16 wherein the primer paint is a zinc primer paint.

18. In the processing of a metal workpiece to form a fabricated article, the steps of claim 15 wherein a welding operation is performed on the deformed workpiece as a finishing operation without first removing residual amounts of said adherent film remaining on the deformed workpiece.

#### References Cited

#### UNITED STATES PATENTS

|           |         |                 |         |   |
|-----------|---------|-----------------|---------|---|
| 2,520,356 | 8/1950  | Bishop          | 117-134 | X |
| 2,774,684 | 12/1956 | Fucinari        | 117-134 | X |
| 2,966,425 | 12/1960 | Fucinari et al. | 117-134 | X |
| 2,976,179 | 3/1961  | Westlund        | 117-134 | X |

RALPH S. KENDALL, Primary Examiner.

ALFRED L. LEAVITT, Examiner.